

Patented Nov. 15, 1927.

1,649,710

# UNITED STATES PATENT OFFICE.

HANS LEEMANN, OF BOTTMINGERMUHLE-BINNINGEN, NEAR BASEL, AND GIOVANNI TAGLIANI, OF BASEL, SWITZERLAND, ASSIGNEES, BY MESNE ASSIGNMENTS, TO MUNITEX CORPORATION, OF LODI, NEW JERSEY, A CORPORATION OF NEW JERSEY.

## RESERVE DYEING ON VEGETABLE FIBERS.

No Drawing. Application filed April 27, 1925, Serial No. 26,289, and in Germany May 7, 1924.

The hitherto known reserve processes consist of mechanical or chemical operations. To the first type belongs the binding and the covering of the vegetable fibers (yarns and fabrics) by substances insoluble in water so that the dyestuffs employed can only soak in and be fixed on the unbound or uncovered parts of the fabric. To the second class belongs the application of certain agents, preferably of salts, which react chemically during the dyeing or during the development of the dyes. All these processes depend, however, on certain conditions. If the reserve agents employed are removed during the dyeing process or during the development of the dyes, when they do not resist these operations until the end of the dyeing, then the desired reserve effect does not occur and the fabric is dyed uniformly throughout as if the reserve means had not been used at all.

It is known from German specification No. 346,883 and others, that it is possible to render vegetable fibers (yarns, loose material, fabrics) completely immune against substantive dyestuffs by treating them after alkalization with solutions of aromatic carboxylic acid chlorides or aromatic sulpho-acid chlorides. Both the alkalization and the action of the aromatic acid or sulpho-acid chlorides are so effected that the whole of the vegetable fibers is brought into the solutions of the respective agents.

It has now been shown in a surprising manner that this esterification can also be used for the topical alteration of the vegetable fibers, in view of the production of reserve effects, for example in a suitable printing process. It was not at all to be foreseen from the more active treatment in solution that the short superficial and sparse local treatment, as it takes place for example in the printing process, would suffice to produce the desired esterification. This process affords permanently reserving patterns with unexpected dyeing properties, which remain fast even after hot washing operations, after hot neutral, acid or alkaline dye baths.

The production of such reserve effects is now utilized in the process for reserve dyeing on vegetable fibers forming the subject of the present invention. This process consists in first treating topically the vegetable fibers by a local printing with a suit-

able alkalizing agent, such for example as a concentrated alkaline solution, with or without thickening agent, with or without the addition of alcohol or with an alcoholic solution of an alkali alcoholate, then in applying thereon in dry or moist condition, an esterifying aromatic acid chloride, such as an aromatic carboxylic acid chloride, or an aromatic sulpho-acid chloride, in pure or dissolved condition, and finally after the resulting esterification in thoroughly washing the vegetable fibers being thus locally altered at the places of the aforesaid print, to constitute what is commonly termed as reserve effects. Thereupon the fibers are dyed with a substantive dyestuff, without the locally altered esterified places taking up the dye, so that they appear white on a colored ground. The fibers may be in form of loose material, yarns or fabrics.

It has also been found that by adding an excess of certain dyestuffs to the alkalizing agent and after treatment with the esterifying agent, colored reserve effects can be obtained on the fibers, which are in no way affected by the subsequent dyeing operations.

Locally esterified vegetable fibers (loose material and yarns) can also be worked up with woollen fibers for mixed fabrics. If these mixed fabrics are first dyed with a basic dyestuff and subsequently in a bath with substantive and certain acid dyestuffs, a special mottled effect can be obtained. The first used basic dyestuff is fixed by the esterified places of the vegetable fibers, the substantive dyestuff by the unaltered vegetable fibers, whilst the woollen material takes up the acid dyestuff.

As dyestuffs, there may be used in all above operations the usual coloring matters which are suitable for carrying out the improved process.

### What we claim is:

1. A process for reserve dyeing on vegetable fibers, which consists in treating topically the vegetable fibers by a local printing with an alkalizing agent, thereupon applying an esterifying aromatic acid chloride to produce a topical alteration of the thus locally printed fiber, then washing subsequently to the esterification and finally dyeing the unaltered vegetable fibers.

2. A process for reserve dyeing on vegetable fibers, which consists in treating topi-

cally the vegetable fibers by a local print-  
ing with an alkalizing agent, thereupon ap-  
plying an esterifying aromatic acid chloride  
to produce a topical alteration of the thus  
5 locally printed fiber, then washing subse-  
quently to the esterification and finally dye-  
ing the unaltered vegetable fibers with a sub-  
stantive dyestuff.

3. A process for reserve dyeing on vege-  
10 table fibers, which consists in treating topi-  
cally the vegetable fibers by a local printing

with an alkalizing agent, thereupon apply-  
ing an esterifying aromatic sulpho-acid chlo-  
ride to produce a topical alteration of the  
thus locally printed fibers, then washing 15  
subsequently to the esterification and finally  
dyeing the unaltered vegetable fibers.

In witness whereof we have hereunto  
signed our names this 15th day of April,  
1925.

HANS LEEMANN.  
GIOVANNI TAGLIANI.